

June 29, 1937.

W. G. D. ORR

2,085,384

CUSHION SHEET

Filed Sept. 1, 1936



INVENTOR  
*William G. D. Orr*  
BY  
*Robert W. Byrly*  
ATTORNEY

## UNITED STATES PATENT OFFICE

2,085,384

## CUSHION SHEET

William G. D. Orr, Chicago, Ill., assignor to A. B.  
Dick Company, Chicago, Ill., a corporation of  
Illinois

Application September 1, 1936, Serial No. 98,866

2 Claims. (Cl. 41—3.5)

This invention relates to cushion sheets for use in stencil-sheet assemblies, and aims to facilitate the cutting of stencils.

Two difficulties have been encountered in preparing stencils by cutting an ordinary stencil sheet on a typewriter. One is danger of cutting out the loop letters, and the other is difficulty in reading the words or marks which have been typed. To avoid these difficulties, stencil-sheet assemblies have been provided in which a cushion sheet is inserted between a stencil sheet and a backing sheet to cushion the blows of the type and to make the typing visible. The requirements for good cushioning and good visibility are, however, so antagonistic that, so far as I am aware, there has been no stencil-sheet assembly which can provide both satisfactory cushioning and visibility like that of ordinary typewriting, although each one of these desiderata has been attained separately without the other.

By my invention, I have provided a new cushion sheet which yields sufficiently under the blows of the typewriter to prevent the type from cutting the fibres of the base of the stencil sheet, and at the same time makes the portions of the stencil sheet which have been struck by the type appear as dark lines against a light background providing a visibility like that attained in ordinary typewriting. I have obtained this result by placing between a stencil sheet and its backing a porous and resilient cushion sheet carrying a small quantity of removable material of a color contrasting with the color of the stencil sheet and the color of the backing. To obtain the fullest advantage of my invention, the stencil mass of the stencil sheet is made white by incorporating a white pigment in it; the backing sheet is of a white or light color; and the cushion sheet has a dark color such as dark blue. In this assembly, the stencil sheet may be of ordinary construction consisting of a base sheet of open, porous paper, such as yoshino paper, carrying a removable stencil mass or impregnating material which weighs several times the weight of the paper and completely fills its interstices. A white or light-colored pigment is preferably incorporated in the stencil mass. My new cushion sheet also includes a base sheet of porous and resilient paper such as yoshino. It carries a removable colored material most desirably consisting of a pigment and a vehicle therefor. The amount of colored material carried by the yoshino paper of the cushion sheet is many times less than the amount of removable material with which the

yoshino paper of the stencil sheet is impregnated. The removable material of the cushion sheet weighs less than the weight of the yoshino paper to which it is applied—preferably less than one-half the weight of the yoshino paper. It adheres to the fibres of the yoshino paper, but is insufficient to fill the interstices between them, and consequently it does not alter the normally porous and resilient character of the yoshino paper.

I have found that typing on such a stencil-sheet assembly has the peculiar effect of causing an interchange of position between the white or light-colored mass on the stencil sheet and the dark-colored material on the cushion sheet. While a part of the stencil mass is forced into the cushion sheet, at the same time dark-colored material from the cushion sheet enters the openings formed in the stencil mass on the stencil sheet by the type, with the result that after typing the stencil sheet presents dark letters against a white background. Furthermore, a part of the dark-colored material in the cushion sheet is driven out upon the backing sheet, so that after typing the backing sheet also presents dark letters on a light background which may be used in proof-reading. Perfect visibility is thus attained both on the stencil sheet itself and on the backing sheet.

Since the dark-colored material of the cushion sheet, although sufficient to have the effects above described, does not fill the interstices between the fibres of the yoshino paper or substantially alter the normal, porous and resilient character of this paper, the cushion sheet is effective to cushion the blows of the type and prevent the type from cutting the fibres of the base of the stencil sheet.

A specific stencil-sheet assembly including a cushion sheet embodying my invention is shown in the accompanying drawing wherein parts are broken away and parts are magnified. In the drawing, A indicates a stencil sheet consisting of a base A<sub>1</sub> of yoshino paper impregnated with a stencil mass A<sub>2</sub> which weighs several times the weight of the paper and completely fills the interstices between the fibres of the paper. The stencil mass may consist of nitrocellulose and a tempering agent, and is given a white color by a white pigment such as lithopone. Eleven per cent. of this material may be incorporated in the stencil mass, as in white stencil sheets heretofore made.

B indicates a cushion sheet consisting of a sheet of yoshino paper B<sub>1</sub> whose fibres carry a

5

10

20

25

30

35

40

45

50

55

small quantity of a removable dark-colored material B2. This material weighs slightly less than one-half the weight of the yoshino paper and leaves the interstices of the paper open.

5 C indicates an ordinary light-colored backing sheet which may consist of manila paper.

The cushion sheet B is prepared by impregnating a sheet of yoshino paper with a liquid of the following composition:

|               | Parts by weight |
|---------------|-----------------|
| Prussian blue | 4.85            |
| Castor oil    | 6.45            |
| Oxalic acid   | .27             |
| Alcohol       | 88.43           |

10 15 and then allowing the alcohol to evaporate. It will be noted that in this example the Prussian blue is a dark-colored pigment, the castor oil is a permanent oily vehicle for the pigment, the alcohol is a volatile solvent or dispersing agent which serves to distribute the pigment and vehicle on the yoshino paper and then evaporates, and the oxalic acid is a peptizing agent which secures even distribution of the pigment.

20 25 The use of a large proportion of volatile dispersing agent, which amounts in the example given to nearly ninety per cent. of the whole impregnating liquid, results in the deposit of a very

small quantity of the non-volatile ingredients on the yoshino sheet. The dark-colored material (Prussian blue and some castor oil) remaining on the yoshino sheet after the evaporation of the alcohol amounts in weight to four-tenths the weight of the yoshino sheet.

5 10 The invention is by no means limited to the particular formula given by way of example, since it is apparent that the removable dark-colored material may be formed of other pigments or lakes or with other vehicles, and that distributing agents other than alcohol may be used.

10 15 What I claim is:

1. A cushion sheet for use in a stencil-sheet assembly, comprising an open, porous and resilient paper, and colored matter removably adhering to the fibres of the paper and insufficient in quantity to fill the interstices between the fibres.

15 20 2. An open, porous and resilient cushion sheet for use in a stencil-sheet assembly, comprising open, porous and resilient paper, and colored material removably adhering to the fibres of the paper and insufficient in quantity to substantially alter the normal open, porous and resilient character of the paper.

25 WILLIAM G. D. ORR.